

# UNITED STATES PATENT OFFICE

ROBERT S. FERGUSON, OF WAUKEGAN, AND WILLIAM SCHUMACHER AND WILLIAM TUBMAN, OF CHICAGO, ILLINOIS.

## COMPOUND FOR INSULATING ELECTRIC WIRES.

SPECIFICATION forming part of Letters Patent No. 320,921, dated June 30, 1885.

Application filed February 27, 1885. (No specimens.)

*To all whom it may concern:*

Be it known that we, ROBERT S. FERGUSON, of Waukegan, in the county of Lake and State of Illinois, and WILLIAM SCHUMACHER and WILLIAM TUBMAN, both of Chicago, county of Cook, and State of Illinois, and all citizens of the United States, have invented a certain new and useful Compound for Insulating Electric Wires, of which the following is a specification.

The object of this invention is to produce a compound containing pine pitch, which shall normally be maintained flexible when cold to a degree effectually preventing said compound from cracking, which compound shall also normally contain sufficient moisture to absorb and carry off induction between two or more wires laid in it, but separated from each other.

Our compound consists of pine-pitch, three hundred (300) pounds; hard or soft rubber, one and one-half ( $1\frac{1}{2}$ ) pound; and liquid asbestos, one (1) gallon, to which is added beeswax, or tallow, or linseed-oil until of the proper consistency to render the compound (when cool) quite hard and yet flexible. To combine these ingredients, they are placed in a suitable vessel, and heated in any desired manner under agitation sufficient to thoroughly mix them.

The essential materials of our compound are pine-pitch and beeswax, or tallow, or linseed-oil, or any similar substances, and in such proportions as will render the pine-pitch (when cool) flexible to a degree sufficient for preventing the pitch from cracking when subject to strains—such, for example, as the bending of

a coated wire, or as occur at the joints of sectional underground conduits—and which will also contain or absorb moisture sufficient to carry off but not promote induction.

In practice any grease, fats, or oils are perhaps preferable to beeswax; but the latter may be used to a very good advantage.

Electric wires simply coated and not embedded in this compound, as they will be when used in underground systems, may, as has been practically demonstrated, be laid in water or on the ground, or both, and yet successfully operate, although only covered by a very thin coat, applied by passing the wire through the compound while in a heated or liquid condition.

What we claim, and desire to secure by Letters Patent, is—

1. The herein-described compound for insulating electric wires, the same consisting of a base composed of pine-pitch and beeswax, or tallow, or linseed-oil, or other materials holding moisture in suspension and rendering the pitch flexible when cool.

2. The herein-described compound for insulating electric wires, the same consisting of pine-pitch, rubber, and asbestos, mixed with beeswax, or tallow, or linseed oil in the manner and proportions specified.

ROBERT S. FERGUSON.

WILLIAM SCHUMACHER.

WM. TUBMAN.

Witnesses:

W. W. ELLIOTT,

JNO. G. ELLIOTT.